

Jan. 24, 1933.

J. B. TYTUS

1,895,299

ROLLING SHEET METAL

Filed Oct. 20, 1927



INVENTOR.

*John B. Tytus*

BY

*Allen Allen*

ATTORNEYS

## UNITED STATES PATENT OFFICE

JOHN B. TYTUS, OF MIDDLETOWN, OHIO, ASSIGNOR TO THE AMERICAN ROLLING MILL COMPANY, OF MIDDLETOWN, OHIO, A CORPORATION OF OHIO

## ROLLING SHEET METAL

Application filed October 20, 1927. Serial No. 227,600.

My invention relates to a process for rolling sheet metal in which sheets of a wide variety of gauges are produced using the Welsh system of rolling or tin mill rolling practice in the finishing, but in which the packs are formed from thin plate produced in a continuous manner.

In my application for Letters Patent Serial No. 21,661, filed April 8, 1925, I explain a process wherein using the principle of the rolling of metal with convexity developed in the piece, which convexity is reduced in each pass, thin plates are formed, which are selected for convexity, matched, heated and rolled into thin sheets.

My present process contemplates a variation over the application for patent above referred to, which is based on refining the operation to the end of assuring packs for the final rolling which are of a type which can be made definite in contour, thus rendering the rolling operation simple.

## In the drawing:—

Figures 1 and 2 are diagrams of a plant for the production of sheet metal according to my invention, in plan and elevation.

In the particular design shown, the roll stands 1, 2, 3 and 4 are formed four high, and the rolls between which the piece passes will be of relatively small diameter, with large diameter backing rolls, which large diameter rolls are held in roller bearings, and the small diameter rolls driven by a suitable series of motors. This mill of four stands is adapted to receive a hot thick slab, and reduce it without cross cutting to a long, wide, thin strip, which is of a width that can be sufficient to satisfy sheet mill requirements.

At 5 I have indicated a set of four high cold rolls, the mill of a single stand being similar in nature to the stands in the hot mill. There may be several stands of these cold rolls if required.

As has been developed by me, the system of roll control in effecting by a continuous roll reduction the attenuation of wide pieces of metal to thin plate or sheet gauges, must be such that the first pass of a series of passes which acts upon the metal just before it has reached a thinness that will inhibit lateral

flow of metal in the pass, will give a convexity to the piece. This convexity then must be reduced proportionately or substantially so, in each successive pass.

In the four high mill selected for illustration, this convexity principle must be followed, and the final piece must have a convexity (crosswise thereof).

It is not highly practical in a rapid reduction process in hot mill rolling of a piece of a single thickness to fairly thin cross section, to deliver a strip which is fully satisfactory for pack forming material. There are no rolls available which will long withstand the excessive wear resulting from rapid reduction processes. The result is that the piece develops roughness, the rolls "cut out" in the active portions and do not give a piece which is accurate as to gauge and a complete control of the contour of the piece is not always obtained.

In order to obtain plate or sheet bodies which are of a uniform smooth surface and accurate as to gauge, I provide for the cold rolling treatment. Thus, as the long strip, in the particular instance, or the series of short strips in the instance illustrated in my patent application hereinabove referred to, are delivered from the hot mill they are permitted to cool, and are then given a pass or passes between the cold rolls.

The attention to contour in the cold rolls should not be relaxed, and a definite control of the original shape of the rolls, and the composition thereof, and the screw applied thereto, will have to be watched carefully, as well as the shape and composition of the piece being cold rolled, to the end of forming an active pass between the rolls of the cold mill which will give a contour to the piece which has been predetermined, as well as an accurate gauge.

The resulting cold rolled product which will be smooth and accurate may then be cut into shorter lengths, and heated up to hot rolling temperature again, and packs formed of the pieces. A heating point is indicated by the diagram of furnaces at 6.

The severing to length can be after heating, or the matching into packs done before

heating, and the heating can be done singly in a continuous furnace.

The mills 7, 8 and 9 as shown are intended to indicate several stands of rolls which will be operated as individual finishing roll stands, and not in a continuous manner. A set of mills will be required to handle the product of the hot and cold mill. The usual tin mill practice of rolling in pairs, doubling, reheating and re-rolling will be followed in the use of these mills. The packs will be formed of lengthwise sections of the cold rolled pieces so that convexity will be increased in the pack over the convexity of the parts making up the pack.

Instead of this a continuous sheet mill, similar in general design to the mills 1, 2, 3 and 4, could be used.

With the usual system of rolling in the tin mill, sheet bars are provided which are very much thicker and very much shorter than the pieces used in forming my packs. These bars are first rolled in a pair, on a roughing mill, and the resultant rough plate is heated, 20 rolled in a pack of two on the sheet mill, reheated, doubled, rolled again, etc., in any of the modes adapted from the Welsh process of rolling. In my system the packs, when 25 they reach the individual rolling stages for finishing, are already longer than a rough plate pack, and this cuts down the time and the various problems involved in the usual 30 tin mill practice.

Unless the packs, in this instance, were 35 very accurate in gauge, as well as being quite smooth in surface and of known contour, which contour would be communicated to the roller who handled the packs, it would be impractical, if not impossible, for the packs 40 to be rolled without becoming so welded together as to be impossible to strip. It is not fully practical to adapt one set of sheet rolls to a succession of packs which vary in their 45 contour, or for that matter in their gauge, which affects the active pass and hence the contour, but with a steady supply of packs of a known temperature, the elements of which are smooth and of a known contour and gauge, the individual stand roller can 50 readily handle the material.

It will be desirable to refrain from picking the hot rolled material before the cold rolling step indicated so as to leave the hot mill scale. This scale is relied upon by the 55 pack roller to set his pack, and furthermore, will permit of opening the packs particularly when the gauge is thin.

A pack is said to be "set" when, after a pass 60 through the mill, the adjoining component parts adhere to each other over their entire surfaces, but not so strongly as to prevent the opening up of the pack after the rolling without damage to the sheets. A loose pack is 65 a pack in which, after a pass through the mill, there is no adhesion of the parts. Both loose

packs and set packs are successfully rolled under different conditions. An intermediate condition is found in "patched packs" in which the adherence of adjoining parts is irregular and incomplete over their areas. The effect 70 of patches is unequal elongation of the component parts in the patched area. Such unequal elongation causes the welding of component parts, transverse folding called "jumping", or longitudinal folding called 75 "pinching", any one of which ruins the pack. It will be clear that gauge and contour inequalities not only directly tend to cause welding since in reduction the pressure is unequally distributed and excessive in parts, 80 but also tend to cause patching and the difficulties, including welding, which flow therefrom.

My process is particularly adapted to the use of strip produced in a continuous mill, as 85 indicated in the drawing, because it is much easier to control the gauge and contour in the slower operating tandem mill, with intermediate shearing, as in my former processes. The intermediate cold rolling step is, however, quite valuable in the second case, as well 90 as in the first, as has been stated.

In either instance the finishing roller need not depart from his regular practice in sheet or tin rolling in which he rolls the pack repeatedly through the individual mills, except to omit the steps of reducing the pair of sheet bars and giving a preliminary reduction to the pack formed of the pair. He will indeed be given a simpler problem, because the very 100 best type of pack will be furnished to him for every operation, and he should be able to dispense with one of the final passes because of being able to control his rolls to better advantage.

Having thus described my invention, what I claim as new and desire to secure by Letters Patent is:—

1. That process of rolling sheet metal, which consists in continuously producing single thickness thin plate or sheet metal by rolling the same when hot, letting the piece cool, giving the piece a cold rolling, in which definite gauge and good surface of the cold rolled piece is assured, the contour of the cold 110 rolled piece being one in which there is a convexity of cross section of the cold rolled piece, and then heating and forming packs of the product, and finally reducing the hot 115 packs to finished gauge by the use of a single stand of rolls which repeatedly acts on each pack.

2. That process of rolling sheet metal, which consists in continuously producing single thickness thin plate or sheet metal by 125 rolling the same when hot, said piece being reduced from the slab without cross cutting, as in strip rolling, letting the piece cool, giving the piece a cold rolling, in which definite gauge and good surface of the cold rolled 130

piece is assured, the contour of the cold rolled piece being one in which there is a convexity of cross section of the cold rolled piece, and then heating and forming packs of the product, and finally reducing the hot packs to finished gauge.

JOHN B. TYTUS.